

1

2,918,414

## ANTIMONY PLATING PROCESS

Glenn R. Schaer, Columbus, Ohio, assignor, by mesne assignments, to Bradley Mining Company, San Francisco, Calif., a corporation of California

No Drawing. Application August 17, 1956  
Serial No. 604,593

6 Claims. (Cl. 204—29)

This invention relates to a process for the deposition of metallic coatings on metal surfaces. More particularly, it relates to the electrodeposition of adherent and continuous coatings of antimony on steel.

It is an object of this invention to deposit antimony coatings on steel directly, without an intermediate coating of another metal. Another object is to deposit the coating of antimony directly on the steel without roughening the surface of the steel previous to the coating, and thereby to produce a smooth coating. A further object is to apply an antimony coating on low-carbon steel continuously and completely over the steel surface. A still further object is to provide a method of coating steel directly from weak antimony acid plating baths.

With the exception of copending patent application, Serial No. 604,630, insofar as is known, no entirely satisfactory method of coating antimony on steel has been found. While certain patents in the prior art allude to successful methods of coating with antimony directly, these methods require the utilization of strongly corrosive antimony fluoride acid solutions and are therefore not completely satisfactory. Patent 2,683,114 is representative of the prior art in this respect. When these prior art methods are used to plate antimony directly on steel, the method calls for roughening the steel by sandblasting or etching processes.

Other prior art methods also disclose the more common method of antimony plating, in which a coating of another metal, such as copper, zinc, or other nonferrous metal, is coated on the steel object prior to the antimony plating operation.

In the process of this invention, the antimony plating may be carried out in a weak citric or other aliphatic hydroxy carboxylic acid bath directly on an unroughened and polished steel object because of the treatment previously given to the surface of the object. The antimony plate produced by the method of this invention is strongly adherent and may be easily buffed to a high polish. In addition, the antimony plate is continuous, covering the exposed surface completely without leaving unplated spots.

Briefly, the process of this invention includes a new process step immediately prior to the antimony plating step. This new process step is the anodic treatment of the object to be coated in an acid solution for a short time at a current density sufficient to cause polarization at the anode object and passivation with the consequent liberation of gas therefrom. The anodic acid treatment step is immediately followed with a rinse step and the antimony plating operation.

While the reasons for the success of this coating process are not definitely known, it is believed that the anodic acid treatment step leaves a chemically uniform surface over all areas of the object and the successful continuous adherence of antimony directly on steel requires such a chemically uniform surface. Objects on which a coating of antimony has been applied directly without the benefit of the new anodic acid treatment have been found to

2

have many dispersed, randomly positioned, unplated spots on the surface. In the electroplating operation, it has been observed that those areas which will receive antimony plate will commence to plate in the very first few seconds after the current is turned on. However, those nonreceptive spots will be immediately apparent, and continued time in the plating operation will not cause any deposit on these spots. It is believed that the reason for the nonreceptive spots may be the existence at these positions of a greater overvoltage for the antimony than the overvoltage for hydrogen in the plating bath. It is thought that the provision of the anodic acid treatment previous to the plating operation reduces the overvoltage of the antimony at these spots to a value less than the overvoltage for hydrogen in the plating bath and that a chemically uniform surface results, making possible the continuous, over-all antimony plating.

In the operation of the method of this invention, certain mineral acids have proved to be effective acid solutions. Sulfuric, phosphoric, and hydrochloric acid solutions have all been used.

A mixture of about 24 to 62 percent by weight sulfuric acid with water has been found to give good direct antimony plating results.

A mixture of about 53 to 85 percent by weight phosphoric acid with water has also been found to give good results.

In addition, a mixture of about 26 to 37 percent by weight hydrochloric acid with water has been found to give good results.

The operating temperature and concentration of the treating solution determine the current density required. In the process, the current density must be high enough to cause polarization of the anode object and passivation with the consequent liberation of gas from the object. At normal room temperatures, successful treatments have been carried out at a current density of about 75 amperes per square foot with solutions in the higher concentration range, for instance, 62 percent for sulfuric acid; 85 percent for phosphoric acid; and 37 percent for hydrochloric acid. At the lower concentrations, and at room temperature, successful treatments have been made at a current density of 100 amperes per square foot.

The time required for the anodic acid treatment is preferably about two minutes. At the usual current densities, bath temperature, and acid concentrations, described above, between 1 and 30 seconds is required to produce polarization at the anode object. Passivation with the consequent liberation of gas, probably oxygen, follows shortly thereafter. The process must be carried on for a sufficient length of time to cause gas liberation. Once the passivation occurs at the anode object, the process may be stopped. However, it is preferred that the process be continued for up to a total of 2 minutes. The process may be continued even longer, and a period of up to 5 minutes may be used to insure treatment over all surfaces of an intricately shaped object. Treatment of longer than 5 minutes appears to be wasted, as no further effect has been found after 5 minutes.

While the exact nature of the surface of the object just previous to, during, and immediately after the commencement of gas liberation is not known, it is believed that the surface may be pure iron and that the treatment may remove most other impurities from the surface and leave a layer one atom thick of iron. The liberation of gas, which is probably oxygen, may leave this surface with an absorbed layer of oxygen on it. It has been found that, after the passivation of the steel object occurs, substantially no iron dissolves. Thus, the physical condition of the surface of the object, such as the roughness thereof, is not disturbed, for all practical

purposes, by the anodic acid treatment process of this invention.

*Example I*

A typical plating process of 4 x 6-inch flat steel panels, in which the anodic acid treatment is combined, is as follows:

(1) The object to be coated is cleaned in a conventional alkaline cleaner solution.

(2) The object is rinsed in water.

(3) The object is immersed or dipped in an acid bath to remove oxide, smut, and other surface impurities. Either sulfuric or hydrochloric acid may be used.

(4) The object is rinsed in water.

(5) The object is connected as the anode in an acid solution of about 53 percent by weight  $H_3PO_4$ . The treatment is conducted for two minutes with the acid at a temperature of between 70 and 90° F. at a current density of about 100 amperes per square foot.

(6) The object is rinsed in water.

(7) The object is electroplated in a citric acid bath of the following composition and under the following operating conditions:

Composition:

|                                                 |       |     |
|-------------------------------------------------|-------|-----|
| Potassium citrate ( $K_3C_6H_5O_7 \cdot H_2O$ ) | g./l. | 145 |
| Citric acid ( $H_3C_6H_5O_7$ )                  | g./l. | 185 |
| Antimony oxide ( $Sb_2O_3$ )                    | g./l. | 60  |
| Water, to make one liter.                       |       |     |

pH 3.5-3.7

Operating conditions:

|                         |              |          |
|-------------------------|--------------|----------|
| Temperature             | °F.          | 120      |
| Anodes                  |              | Antimony |
| Cathode current density | amp./sq. ft. | 30       |

*Example II*

A typical plating process on an intricately shaped steel object, in which the anodic acid treatment step is combined, is as follows:

(1) The object to be plated is cleaned in a conventional alkaline cleaner solution.

(2) The object is rinsed in water.

(3) The object is immersed or dipped in an acid bath to remove oxide, smut, and other surface impurities.

(4) The object is rinsed in water.

(5) The object is connected as the anode in an acid solution of 62 percent by weight  $H_2SO_4$  with water. The treatment is conducted for 5 minutes with the acid at a temperature of between 70 and 90° F. at a current density of about 75 amperes per square foot.

(6) The object is rinsed in water.

(7) The object is electroplated in a citric acid bath of the composition and under the operating conditions described in Example I.

It has been found that mixtures of the three above-described mineral acids may be used if the strength of the individual acid in the solution does not exceed the maximums set forth herein. The ability to mix the acids provides further flexibility in the operation of the process.

Normal brightening agents conventionally used in plating baths are not affected by the anodic treatment of this invention.

One of the advantages to be found in the process of this invention is in the successful treatment at normal room temperatures. It is apparent that any process operation which may be carried out at normal ambient temperatures is better than similar processes which must be operated at elevated temperature because there is no need for temperature control and heat-addition or subtraction apparatus. Of course, continued use of the bath may raise the bath temperature because of the resistance of the solution to current passage. This increase in temperature has no detrimental effect on the operation, except to require higher current densities. However, the ability to operate initially at room temperature is a con-

venience, and an economic factor in the favor of room-temperature operation.

An additional advantage to be found in the process of the invention is the use of relatively dilute acids. The use of dilute acids results in there being less effect on the strength of the treating bath by water transmittal from the cleaning solution and the rinsing bath. In any plating operation, there is the problem of carry-over from one solution to the next in the successive dipping operations. In addition, the use of dilute acids provides better control over the operation, in that the treating solution, if sulfuric acid is used, does not change its strength because of hydroscopic absorption from the air.

In view of the fact that the three separate acids—sulfuric, phosphoric, and hydrochloric—have been found to give good treating results in preparing a steel object for antimony plating, the plating operation is provided with flexibility that is advantageous. The particular treating solution may be selected on the basis of its compatibility with the plating bath. Therefore, any carry-over from the treating solution through the rinsing solution to the plating solution by the successive dipping process will not harm the plating bath.

In the prior art method of coating antimony on steel by means of strongly corrosive antimony fluoride acid baths, the corrosive nature of the plating bath is a decided disadvantage. The use of such highly corrosive acids makes necessary the provision of expensive ventilating and handling equipment. This invention, by making possible the use of weak aliphatic hydroxy carboxylic acids eliminates these problems.

In the prior art methods of plating antimony directly on steel by strong antimony fluoride acid solutions, there is also the disadvantage that these acid solutions attack the object to be plated during the early stages of the plating operation before the object is covered with antimony plate, and, therefore, there is a loss of metal from the object and contamination of the plating bath.

In the prior art methods of coating antimony on steel by means of intermediate coatings, it has been found that intermediate coatings, such as copper and zinc, form alloys with antimony, by room-temperature diffusion, and that these alloys are brittle and cause the plated coatings to peel. Direct coatings by the method of this invention have been formed to an angle of 180 degrees after being stored for six months, and the coatings have been found to be pliable with no tendency to peel.

It has been found that electropolishing will also condition the surface of a steel object to accept antimony plating. However, the electropolishing operation removes metal but the anodic treatment process does not. Of course, in a process which removes metal, there is the disadvantage of bath contamination caused by the metal which is successively removed from the succeeding objects; in addition, when the contamination builds up in the electropolishing bath, the iron salts will often be carried into the antimony plating bath in a normal, successive-dipping cycle.

It will be understood, of course, that while the forms of the invention herein shown and described constitute preferred embodiments of the invention, it is not intended herein to illustrate all of the possible equivalent forms or ramifications of the invention. It will also be understood that the words used are words of description rather than of limitation and that various changes may be substituted without departing from the spirit or scope of the invention herein disclosed.

What is claimed is:

1. The process of preparing a steel object to receive an electrodeposited coating of antimony comprising: preceding the application of said antimony on said steel object by treating said steel anodically in an acid solution at a current density of at least about 75 amperes per square foot for a sufficient length of time to cause passivation at said anodic object with consequent liberation

of gas therefrom, the physical condition of the surface of said object not being disturbed thereby; said acid being selected from the group consisting of sulfuric acid, phosphoric acid, and hydrochloric acid.

2. In the process of plating antimony on a steel object comprising cleaning said steel object followed by a first rinsing operation, acid dipping said steel object followed by a second rinsing operation, and electroplating said steel object with antimony; the step following said second rinsing operation of treating said steel object anodically in an acid solution, at normal room temperature at a current density of from about 75 to 100 amperes per square foot for sufficient length of time to cause passivation at said anodic object with consequent liberation of gas therefrom, the physical condition of the surface of said object not being disturbed thereby; said acid solution being selected from the group consisting of sulfuric acid, phosphoric acid, and hydrochloric acid.

3. The process of electrodepositing antimony on a steel object comprising: cleaning said steel object in an alkaline cleaning solution; rinsing said steel object; treating said steel object in an acid dip; subjecting said steel to a second rinse; treating said steel object anodically in an acid solution, wherein said acid is selected from the group consisting of sulfuric acid, phosphoric acid, and hydrochloric acid, for a period of between 1 and 300 seconds at normal room temperature, and at a current density of from 75 to 100 amperes per square foot, said period being a sufficient length of time to cause passivation at said anodic object with consequent liberation of gas therefrom, the physical condition of the surface of said object not being disturbed thereby; subjecting said steel to a third rinse; and electroplating antimony on said steel in an aliphatic hydroxy carboxylic acid plating solution.

4. A process of preparing steel for the electro-deposition of antimony coatings thereon comprising: preceding the application of said antimony on said steel by treating said steel anodically in a sulfuric acid solution of about 62 percent by weight at a temperature of between 70 and 90° F. for a period of between 1 and 300 seconds at a current density of about 75 amperes per square foot, said anodic treatment causing passivation

at said anodic object with consequent liberation of gas therefrom, the physical condition of the surface of said object not being disturbed thereby.

5. A process of preparing a steel object for the electro-deposition of antimony coatings thereon comprising: preceding the application of said antimony on said steel object by treating said steel object anodically in a solution of about 85 percent by weight phosphoric acid at a temperature of between 70 and 90° F. for a period of between 1 and 300 seconds at a current density of about 75 amperes per square foot, said anodic treatment causing passivation at said anodic object with consequent liberation of gas therefrom, the physical condition of said object not being disturbed thereby.
- 10 15 6. A process of preparing a steel object for the electro-deposition of antimony coatings thereon comprising: preceding the application of said antimony on said steel object by treating said steel object anodically in a solution of about 37 percent by weight hydrochloric acid at a temperature of between 70 and 90° F. for a period of between 1 and 300 seconds at a current density of about 75 amperes per square foot, said anodic treatment causing passivation at said anodic object with consequent liberation of gas therefrom, the physical condition of the 20 25 surface of said object not being disturbed thereby.

#### References Cited in the file of this patent

#### UNITED STATES PATENTS

- |    |           |                         |               |
|----|-----------|-------------------------|---------------|
| 30 | 2,569,453 | Chester et al. -----    | Oct. 2, 1951  |
|    | 2,721,836 | Du Rose -----           | Oct. 25, 1955 |
|    | 2,748,066 | Whitehouse et al. ----- | May 29, 1956  |
|    | 2,750,333 | Smart -----             | June 12, 1956 |

#### FOREIGN PATENTS

- |    |         |                     |              |
|----|---------|---------------------|--------------|
| 35 | 559,164 | Great Britain ----- | Feb. 7, 1944 |
|----|---------|---------------------|--------------|

#### OTHER REFERENCES

Principles of Electroplating and Electroforming, 3rd edition, Blum and Hogaboom, McGraw-Hill Book Company, Inc., New York, 1949.

Modern Electroplating, edited by A. G. Gray, John Wiley & Sons Inc., New York, 1953, pp. 486 and 487.